# EUROPEAN PATENT SPECIFICATION

(11) **EP 2 314 840 B1**
(45) Date of publication and mention of the grant of the patent: **23.05.2012**
(21) Application number: 10187419.6
(22) Date of filing: 13.10.2010
(51) Int. Cl.: F01N 13/14

(54) **Heat insulator for a vehicle exhaust pipe, vehicle pipe and methods for manufacturing the same**
Wärmeisolierung für eine Fahrzeugabgasleitung, Fahrzeugleitung und Verfahren zu deren Herstellung
Isolant thermique pour tuyau d'échappement de véhicule, tuyau de véhicule et procédés pour leur fabrication

(30) Priority: 20.10.2009 JP 2009240964
(43) Date of publication of application: 27.04.2011
(73) Proprietor: Nakagawa Sangyo Co., Ltd., Inuyama-shi, Aichi (JP)
(72) Inventor: Nakagawa, Noriaki, Inuyama-shi Aichi (JP)
(74) Representative: Kramer - Barske - Schmidtchen

(56) References cited:
- EP-A1- 1 617 126
- JP-A- 10 196 880
- JP-A- 2005 201 458
- US-A- 2 094 334
- US-A- 2 468 589
- US-A- 4 726 974
- US-A- 4 985 106
- US-A- 5 869 407
- US-A1- 2004 253 406
- US-A1- 2009 186 176

## Description

The present invention relates to a heat insulator for a vehicle exhaust pipe, a vehicle exhaust pipe insulated by the heat insulator and methods for manufacturing the heat insulator and the vehicle exhaust pipe insulated by the heat insulator.

A catalytic converter for purifying exhaust gas is typically installed in an exhaust pipe of a vehicle and the catalyst used in the catalytic converter is typically activated at a temperature of 300°C or higher. Thus, after starting up the engine, it is necessary to rapidly increase the temperature of the catalyst to 300°C or higher in order to promptly start the exhaust gas purification. For environmental reasons, the light-off time, i.e. the period of time after engine ignition until the catalyst is activated, has recently been set to an extremely short time and thus there is a need to supply the engine exhaust gas to the catalytic converter without reducing the temperature of the engine exhaust gas so as to promptly activate the catalyst.

One way to prevent the temperature of the engine exhaust gas from undesirably decreasing is to provide a heat insulator around the exhaust pipe so as to extend from the engine to the catalytic converter. As disclosed, e.g., in Japanese Laid-Open Patent Publication No. 09-151730, a heat insulator is proposed that has a structure in which a glass wool mat is wound around an outer periphery of the exhaust pipe and the glass wool mat is then covered by an outer pipe. Thus, a heat insulator is proposed that, when combined with the exhaust pipe, has a double pipe structure in which an air layer is formed around the outer periphery of the exhaust pipe.

US 5,869,407 A relates to a fibrous insulation product having inorganic binders.

US 2004/253406 A1 discloses a vacuum heat insulating material and a manufacturing method thereof.

US 2,094,334 A relates to a heat insulating tape.

US 2,468,589 A discloses an insulating tape.

EP 1 617 126 A1 relates to a vacuum thermal insulation material and a device using the same.

US 2009/186176 A1 discloses a vacuum heat insulating material, a method of producing the same and a heat insulating box body using said vacuum heat insulating material.

US 4,985,106 A relates to an insulation structure for appliances.

JP 10-196880 A discloses the manufacture of a vacuum insulation material.

US 4,726,974 A relates to a vacuum insulation panel.

JP 2005-201458 A discloses a vacuum heat insulation material.

However, the above-described known heat insulators still lacks sufficient heat insulating and heat retaining properties. Consequently, a heat insulator is required that has further improved thermal insulation properties so as to reduce the light-off time.

It is an object of the present teachings to provide a heat insulator for a vehicle exhaust pipe capable of reducing the light-off time due to improved thermal insulation properties, to provide a method for manufacturing such a heat insulator, as well as to provide exhaust pipes insulated by such heat insulators.

This object is achieved by the heat insulator of claim 1, the vehicle exhaust pipe of claim 7 and the manufacturing methods of claims 9 and 12. Further developments of the invention are recited in the dependent claims.

According to the heat insulator of claim 1, a vacuum state exists inside the bag member comprised of the heat-resistant metal foil(s) that accommodate(s) the heat insulating material therein. The heat insulator for the vehicle exhaust pipe thus exhibits excellent thermal insulation properties and is capable of reducing the light-off time required to activate the catalyst after engine ignition.

In another aspect of the present teachings, a method for manufacturing such a heat insulator includes positioning the heat insulating material (5) between two heat-resistant metal foil sheets (41 and 42), superimposing the edges of the two metal foil sheets (41 and 42) to enclose the heat insulating material (5), hermetically joining the superimposed edges of the metal foil sheets (41 and 42) except at one portion (4a) to form it into a bag shape that opens at the portion (4a), evacuating the bag comprised of the metal foil sheets (41 and 42) through the opening at the portion (4a), and then closing the opening at the part (4a) by joining so as to form the bag member (4). Stainless steel foil having a thickness of 20 µm to 50 µm is used as the metal foil. A non-woven fabric made of a glass fiber, a basalt fiber and/or a ceramic fiber, is used as the heat insulating material, wherein the heat insulating material has a thickness of 8 to 12 mm.

The reference numeral(s) or the set of reference characters in each pair of parentheses above denotes a correspondence to specific structures disclosed in a representative embodiment that will be further described below.

As was described above, a heat insulator for a vehicle exhaust pipe according to the present teachings is capable of exhibiting excellent thermal insulation properties and may, in certain embodiments, significantly reduce the light-off time required to activate the catalyst after engine ignition. Preferred embodiments of the invention will now be described in further detail with the assistance of the drawings, in which:

FIG. 1 is a schematic, partial cross-sectional view of a vehicle exhaust pipe provided with a representative, non-limiting heat insulator;
FIG. 2 is an enlarged cross-sectional view of a peripheral wall portion of the vehicle exhaust pipe provided with the representative, non-limiting heat insulator;
FIG. 3 is a perspective, exploded view showing a step in a representative, non-limiting process for manufacturing the heat insulator; and
FIG. 4 is a perspective view showing another step in the representative, non-limiting process for manufacturing the heat insulator.

Referring to FIG. 1, a representative heat insulator 1 according to the present teachings is provided around the outer periphery of a vehicle exhaust pipe 2 which is connected to an exhaust manifold E1 of an engine E so as to extend from an upstream end to an inlet of a catalytic converter 3 provided in a middle portion of the exhaust pipe 2. FIG. 2 shows an enlarged cross-sectional view of the heat insulator 1. Each heat insulator 1 includes a bag member 4 having a certain length and being disposed along the exhaust pipe 2. As shown in FIG. 1, a plurality of heat insulators 1 are wound or wrapped around the outer periphery of the exhaust pipe 2 adjacent to each other in a sufficient number so as to cover the entire outer periphery of the exhaust pipe 2 between the exhaust manifold E1 and the catalytic converter 3. A deformable or bendable sheet-shaped heat insulating material 5 (e.g., a heat insulating mat) having a thickness of 8 mm to 12 mm is inserted into each bag member 4 and the inside of the bag member 4 is subjected to a vacuum or reduced pressure state. The plurality of heat insulators 1 having the above-described configuration are retained around the outer periphery of the vehicle exhaust pipe 2 by a metal cover body 6, which covers the respective outer surfaces of the heat insulators 1. It is noted that, if the thickness of the heat insulating material 5 is greater than 12 mm, the evacuation step (to be described below) will require a relative long time. On the other hand, if the thickness is less than 8 mm, the heat insulating effectiveness is impaired.

Each bag member 4 consists of heat-resistant metal foil that is preferably capable of withstanding a high temperature of at least 700 to 800°C. Stainless steel foil having both high corrosion resistance and high heat resistance is used as the metal foil. The thickness of the stainless steel foil is 20 to 50 µm.

For example, a non-woven mat comprising one or more of glass fiber or ceramic fiber exhibiting a low thermal conductivity, is used as the heat insulating material 5. Preferred glass fibers are glass fiber yarns available from Nitto Boseki, headquartered in Tokyo, Japan with a main branch in Fukushima, Japan, under the product name ECG. ECG has the following specifications: filament diameter 9.1 microns, filament count 200 to 800, twist 1.0/25 mm or 0.7/25 mm, Tex 33.7 to 135.0 (g/1000 m) and length per kilogram 7.4 to 29.6 (km/kg).

The degree of the vacuum or reduced pressure state existing in each bag member 4 is preferably set to about 1 to 20 Pa, more preferably 1 to 10 Pa. It is noted that if the thickness of the metal foil is greater than 50 µm, the deformability or bendability of the foil is impaired, and the evacuation requires a relatively long time. On the other hand, if the thickness is less than 20 µm, it becomes difficult to weld or sealingly join the metal foil, as will be further described below.

In one representative method for manufacturing a heat insulator 1 with the above-described configuration, two metal foil sheets 41 and 42 of a predetermined size are prepared and a mat or layer of heat insulating material 5 is inserted between the metal foil sheets 41 and 42, as shown in FIG. 3. After that, three edges of the two metal foil sheets 41 and 42 are joined or sealed by seam welding along three sides, i.e. excluding one side 4a (the joined/sealed portions are indicated by a chain double-dashed line in FIG. 4). Instead of seam welding, microplasma welding or fiber laser welding also may be used.

The metal foil sheets 41 and 42 are joined at the three sides to form a bag-shape. The bag-shape comprised of the metal foil sheets 41 and 42 and containing the heat insulating material 5 is placed in a vacuum chamber and is evacuated to the same reduced pressure existing in the vacuum chamber, preferably about 1 to 10 Pa, through the unjoined ends serving as an opening on the one side 4a. Thereafter, the unjoined side 4a is provisionally closed by heat sealing and the bag-shape is removed from the vacuum chamber. Lastly, the metal foil sheets 41 and 42 are securely or permanently joined or sealed along the provisionally-sealed side 4a by seam welding to form the hermetically sealed bag member 4, thereby completing the heat insulator 1. As was described above, a plurality of thus-obtained heat insulators 1 are preferably wound around the outer periphery of the vehicle exhaust pipe 2 adjacent to each other so as to extend from the exhaust manifold E1 to the catalytic converter 3. The outer circumference of the heat insulators 1 is then covered with the metal cover body 6, which retains the heat insulators 1.

As a particular example, the bag member 4 was prepared using stainless steel foil having a thickness of 50 µm and heat insulating material 5 having a thickness of 8 mm prepared from a non-woven fabric (with a density of 587 g/m²) made of a glass fiber, and the bag member 4 was evacuated to 10 Pa, thereby obtaining the heat insulator 1. The thermal conductivity of the heat insulator 1 having this configuration was measured using a heat flow meter method for a sheet (JIS-A-1412 (1994)) and was determined to be 0.0183 W/(m·K). In contrast, the thermal conductivity of the known heat insulator described in the introductory portion above was measured using the same above-described measurement method and was determined to be 0.032 W/(m·K). As can be seen from this, a heat insulator according to the present embodiment exhibits a thermal conductivity of about one-half of the known heat insulator and thus exhibits excellent thermal insulation properties as compared to the known art. When such a heat insulator is used to insulate a vehicle exhaust pipe, the light-off time can be significantly reduced.

Although the present heat insulators have been directed towards applications involving a vehicle exhaust pipe, it is understood that the heat insulators may be utilized in any application that requires insulating a structure or retaining heat within a structure, e.g., a pipe structure. For example, the present teachings also may be utilized to insulate heating ducts and/or cooling ducts.

## Claims

1. A heat insulator (1) for a vehicle exhaust pipe (2) which is windable around an outer periphery of the vehicle exhaust pipe, the heat insulator comprising a deformable sheer-shaped heat insulating material (5) hermetically encased in a reduced pressure state in a bag member (4) consisting of a heat-resistant metal foil (41, 42), which is a stainless steel foil having a thickness of 20 µm to 50 µm, wherein the heat insulating material (5) consists of a non-woven fabric consisting of a glass fiber, a basalt fiber and/or a ceramic fiber, and wherein the heat insulating material (5) has a thickness of 8 to 12 mm.

2. The heat insulator according to claim 1, wherein the heat-resistant metal foil (41, 42) is capable of withstanding a temperature of at least 700°C.

3. The heat insulator according to claim 1 or 2, wherein the non-woven fabric consists of a glass fiber yarn having a Tex of 33.7 to 135.0 g/1000 m.

4. The heat insulator according to any preceding claim, wherein the heat insulating material (5) has a density of 550-600 g/m².

5. The heat insulator according to any preceding claim, wherein the reduced pressure state inside the bag member (4) is between 1 to 20 Pa, more preferably between 1 to 10 Pa.

6. The heat insulator according to any preceding claim, wherein the heat insulator exhibits a thermal conductivity of less than or equal to 0.25 W/ (m·K), more preferably less than or equal to 0.20 W/ (m·K).

7. A vehicle exhaust pipe (2) wherein one or more heat insulators (1) according to any preceding claim is wound around its outer periphery.

8. A vehicle exhaust pipe (2) according to claim 7 having a metal cover body (6) disposed around the one or more heat insulators (1).

9. A method for manufacturing the heat insulator according to any one of claims 1-6, comprising:
positioning the heat insulating material (5) between two heat-resistant metal foil sheets (41, 42), which are stainless steel foils having a thickness of 20 µm to 50 µm, wherein the heat insulating material (5) consists of a non-woven fabric consisting of a glass fiber, a basalt fiber and/or a ceramic fiber, and wherein the heat insulating material (5) has a thickness of 8 to 12 mm,
superimposing the edges of the two metal foil sheets to enclose the heat insulating material,
hermetically joining the edges of the metal foil sheets to form a bag-shape while leaving at least one opening (4a),
evacuating the interior of the bag-shape through the opening, and
sealing the opening to form a bag member (4) containing the heat insulating material under reduced pressure.

10. The method according to claim 9, wherein the non-woven fabric consists of a glass fiber yarn having a Tex of 33.7 to 135.0 g/1000 m.

11. The method according to claim 9 or 10, wherein the evacuation step includes reducing the pressure inside the bag shape to between 1 to 20 Pa, more preferably between 1 to 10 Pa.

12. A method for manufacturing the vehicle exhaust pipe (2) according to claim 7, comprising winding one or more heat insulators (1) according to any one of claims 1-6 around the outer periphery of the vehicle exhaust pipe (2).

13. The method according to claim 12, further comprising disposing a metal cover body (6) around the one or more heat insulators (1).

## Patentansprüche

1. Wärmeisolator (1) für ein Fahrzeugabgasrohr (2), der um einen Außenumfang des Fahrzeugabgasrohrs gewickelt werden kann, wobei der Wärmeisolator ein verformbares, blattförmiges Wärmeisoliermaterial (5) umfasst, das in einem Zustand mit vermindertem Druck in einem Beutelelement (4) hermetisch eingeschlossen ist, welches aus einer wärmebeständigen Metallfolie (41, 42) besteht, bei der es sich um eine Folie aus rostfreiem Stahl mit einer Dicke von 20 µm bis 50 µm handelt, wobei das Wärmeisoliermaterial (5) aus einem Vlies besteht, das aus einer Glasfaser, einer Basaltfaser und/oder einer Keramikfaser besteht, und wobei das Wärmeisoliermaterial (5) eine Dicke von 8 bis 12 mm aufweist.

2. Wärmeisolator nach Anspruch 1, bei dem die wärmebeständige Metallfolie (41, 42) einer Temperatur von mindestens 700 °C widerstehen kann.

3. Wärmeisolator nach Anspruch 1 oder 2, bei dem das Vlies aus einem Glasfasergarn mit einem Tex-Wert von 33,7 bis 135,0 g/1000 m besteht.

4. Wärmeisolator nach einem der vorhergehenden Ansprüche, bei dem das Wärmeisoliermaterial (5) eine Dichte von 550 bis 600 g/m² aufweist.

5. Wärmeisolator nach einem der vorhergehenden Ansprüche, bei dem der Zustand mit vermindertem Druck innerhalb des Beutelelements (4) zwischen 1 bis 20 Pa, mehr bevorzugt zwischen 1 bis 10 Pa liegt.

6. Wärmeisolator nach einem der vorhergehenden Ansprüche, wobei der Wärmeisolator eine Wärmeleitfähigkeit von weniger als oder gleich 0,25 W/(m · K), mehr bevorzugt weniger als oder gleich 0,20 W/(m · K) aufweist.

7. Fahrzeugabgasrohr (2), bei dem einer oder mehrere der Wärmeisolatoren (1) gemäß einem der vorhergehenden Ansprüche um dessen Außenumfang gewickelt ist oder sind.

8. Fahrzeugabgasrohr (2) nach Anspruch 7, das einen Metallabdeckungskörper (6) aufweist, der um den einen Wärmeisolator (1) oder die mehreren Wärmeisolatoren (1) herum angeordnet ist.

9. Verfahren zur Herstellung des Wärmeisolators nach einem der Ansprüche 1 bis 6, umfassend:
Positionieren des Wärmeisoliermaterials (5) zwischen zwei wärmebeständigen Metallfolienlagen (41, 42), bei denen es sich um Folien aus rostfreiem Stahl mit einer Dicke von 20 µm bis 50 µm handelt, wobei das Wärmeisoliermaterial (5) aus einem Vlies besteht, das aus einer Glasfaser, einer Basaltfaser und/oder einer Keramikfaser besteht, und wobei das Wärmeisoliermaterial (5) eine Dicke von 8 bis 12 mm aufweist,
Aufeinanderlegen der Kanten der zwei Metallfolienlagen zum Einschließen des Wärmeisoliermaterials,
hermetisches Verbinden der Kanten der Metallfolienlagen zum Bilden einer Beutelform, während mindestens eine Öffnung (4a) freigelassen wird,
Evakuieren des Inneren der Beutelform durch die Öffnung und
Verschließen der Öffnung zum Bilden eines Beutelelements (4), welches das Wärmeisoliermaterial unter vermindertem Druck enthält.

10. Verfahren nach Anspruch 9, wobei das Vlies aus einem Glasfasergarn mit einem Tex-Wert von 33,7 bis 135,0 g/1000 m besteht.

11. Verfahren nach Anspruch 9 oder 10, wobei der Evakuierungsschritt das Vermindern des Drucks innerhalb der Beutelform auf zwischen 1 bis 20 Pa, mehr bevorzugt zwischen 1 bis 10 Pa umfasst.

12. Verfahren zur Herstellung des Fahrzeugabgasrohrs (2) nach Anspruch 7, umfassend das Wickeln eines Wärmeisolators (1) oder mehrerer Wärmeisolatoren (1) nach einem der Ansprüche 1 bis 6 um den Außenumfang des Fahrzeugabgasrohrs (2).

13. Verfahren nach Anspruch 12, das ferner das Anordnen eines Metallabdeckungskörpers (6) um den einen Wärmeisolator (1) oder die mehreren Wärmeisolatoren (1) herum umfasst.

## Revendications

1. Isolant thermique (1) pour tuyau d'échappement de véhicule (2) qui peut être enroulé autour d'une périphérie externe du tuyau d'échappement de véhicule, l'isolant thermique comprenant unmatériau d'isolation thermique (5) en forme de feuille déformable, enserré hermétiquement sous pression réduite dans une poche (4) constituée d'une feuille métallique (41, 42) résistant à la chaleur, qui est une feuille d'acier inoxydable ayant une épaisseur de 20 µm à 50 µm, dans lequel le matériau d'isolation thermique (5) est constitué d'un tissu non tissé formé d'une fibre de verre, d'une fibre de basalte et/ou d'une fibre de céramique et dans lequel le matériau d'isolation thermique (5) a une épaisseur de 8 à 12 mm.

2. Isolant thermique selon la revendication 1, dans lequel la feuille métallique (41, 42) résistant à la chaleur est capable de résister à une température d'au moins 700 °C.

3. Isolant thermique selon la revendication 1 ou 2, dans lequel le tissu non tissé est constitué d'un fil en fibres de verre ayant une unité Tex de 33,7 à 135,0 g/1000 m.

4. Isolant thermique selon l'une quelconque des revendications précédentes, dans lequel le matériau d'isolation thermique (5) a un grammage de 550 à 600 g/m².

5. Isolant thermique selon l'une quelconque des revendications précédentes, dans lequel l'état de pression réduite à l'intérieur de la poche (4) est compris entre 1 et 20 Pa, plus particulièrement entre 1 et 10 Pa.

6. Isolant thermique selon l'une quelconque des revendications précédentes, dans lequel l'isolant thermique présente une conductibilité thermique inférieure ou égale à 0,25 W/(m·K), plus particulièrement inférieure ou égale à 0,20 W/(m·K).

7. Tuyau d'échappement de véhicule (2), dans lequel un ou plusieurs isolants thermiques (1) selon l'une quelconque des revendications précédentes est ou sont enroulés autour de sa périphérie externe.

8. Tuyau d'échappement de véhicule (2) selon la revendication 7, ayant un corps de couverture métallique (6) disposé autour du ou des isolants thermiques (1).

9. Procédé de fabrication de l'isolant thermique selon l'une quelconque des revendications 1 à 6, comprenant :
le positionnement du matériau d'isolation thermique (5) entre deux feuilles de métal (41, 42) résistant à la chaleur, qui sont des feuilles en acier inoxydable d'une épaisseur de 20 µm à 50 µm, dans lequel le matériau d'isolation thermique (5) est constitué d'un tissu non tissé formé d'une fibre de verre, d'une fibre de basalte et/ou d'une fibre de céramique et dans lequel le matériau d'isolation thermique (5) a une épaisseur de 8 à 12 mm,
la superposition des bords des deux feuilles de métal pour enserrer le matériau d'isolation thermique,
la jonction hermétique des bords des feuilles de métal pour donner une forme de poche tout en laissant au moins une ouverture (4a),
l'évacuation de l'intérieur de la poche formée à travers l'ouverture, et
le scellage de l'ouverture pour former une poche (4) contenant le matériau d'isolation thermique sous pression réduite.

10. Procédé selon la revendication 9, dans lequel le tissu non tissé est constitué d'un fil de fibres de verre ayant une unité Tex de 33,7 à 135,0 g/1000 m.

11. Procédé selon la revendication 9 ou 10, dans lequel l'étape d'évacuation comprend la réduction de la pression à l'intérieur de la poche formée à une valeur comprise entre 1 et 20 Pa, plus particulièrement entre 1 et 10 Pa.

12. Procédé de fabrication du tuyau d'échappement de véhicule (2) selon la revendication 7, comprenant l'enroulement d'un ou plusieurs isolants thermiques (1) selon l'une quelconque des revendications 1 à 6 autour de la périphérie externe du tuyau d'échappement de véhicule (2).

13. Procédé selon la revendication 12, comprenant en outre la disposition d'un corps de couverture métallique (6) autour du ou des isolants thermiques (1).
